

# United States Patent Office

2,978,511

Patented Apr. 4, 1961

1

2,978,511

## NITRATE AND PERCHLORATE SALTS OF NITRAZA DIAMINES

Milton B. Frankel, Pasadena, Calif., assignor to Aerojet-General Corporation, Azusa, Calif., a corporation of Ohio

No Drawing. Filed Oct. 25, 1957, Ser. No. 692,964

20 Claims. (Cl. 260—583)

This invention relates to new compositions of matter and a method for their preparation. In particular, the invention relates to bis-inorganic acid salts of nitraza diamines having the general formula



wherein X is a nitrate or perchlorate radical, A and A' are alkylene radicals, and n is a whole number from 1 to 6, inclusive.

Due to their high oxygen content, the nitro compounds of this invention are useful as high explosives and can be used in any conventional explosive missile, projectile, rocket, or the like as the main explosive charge. An example of such a missile is disclosed in U.S. Patent No. 2,470,162, issued May 17, 1949. One way of using the high explosives in a device such as that disclosed in U.S. Patent No. 2,470,162 is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time-fuse mechanism firing a detonating explosive such as lead azide or mercury fulminate.

The compounds of this invention are readily prepared by treating a nitraza diisocyanate with dilute nitric or perchloric acid, in accordance with the general reaction scheme set forth below:



wherein X, A, A', and n are as defined above.

To more fully illustrate this invention, the following examples are presented. It is to be understood, however, that these examples are presented merely as a means of illustration and are not intended to limit the scope of the invention in any way.

### EXAMPLE I

#### Preparation of the bis-nitric acid salt of 3-nitraza-1,5-pentane diamine

In a round bottom flask fitted with a reflux condenser, 3-nitraza-1,5-pentane diisocyanate was heated with a ten-fold excess of 35% nitric acid on a steam bath for a period of 3 hours. The solution was evaporated to dryness in vacuo leaving a quantitative yield of the bis-nitrate salt of 3-nitraza-1,5-pentane diamine. Upon recrystallization from ethyl acetate and ether, the product exhibited a M.P. of 153–155° C. The elemental analysis of the product is as follows:

Calculated for  $\text{C}_4\text{H}_{14}\text{N}_6\text{O}_8$ : percent C, 17.52; percent

2

H, 5.15; percent N, 30.65. Found: percent C, 17.66; percent H, 5.11; percent N, 30.78

The explosive power of this compound was calculated to be:

5 Lead block value 112 TNT=100  
Ballistic mortar value 126 TNT=100

### EXAMPLE II

#### Preparation of the bis-nitric acid salt of 3,6-dinitraza-1,8-octane diamine

The bis-nitric acid salt of 3,6-dinitraza-1,8-octane diamine was prepared by reacting 3,6-dinitraza-1,8-octane diisocyanate with 35% nitric acid according to the procedure described in Example I and recrystallizing the product from methanol. The product exhibited a M.P. of 185–190° C. The elemental analysis of the product is as follows:

Calculated for  $\text{C}_6\text{H}_{18}\text{N}_8\text{O}_{10}$ : percent C, 19.89; percent H, 5.01; percent N, 30.93. Found: percent C, 20.56; percent H, 5.01; percent N, 30.78

The explosive power of this compound was found to be:

25 Lead block value 109 TNT=100  
Ballistic mortar value 125 TNT=100

As indicated above, a dilute acid is employed for the reaction of the present invention. By dilute acid, as the term is employed herein, is meant an aqueous solution of acid, preferably of from about 30 to about 85% concentration. The reaction of this invention is a vigorous one and I have found that optimum control can be exercised when an acid of about 35% concentration is employed in excess. The excess acid acts as a diluent or solvent and thereby effects moderation of the reaction.

30 Reaction temperature is not critical in the practice of this invention, the only effect of temperature variation being a corresponding increase or decrease in reaction rate. I have found, however, that elevated reaction temperatures such as those from ambient to about 100° C. result in particularly favorable reaction rates and that the reaction proceeds most efficaciously at steam bath temperature.

35 The nitraza diisocyanates useful as starting materials for this invention, such as 3-nitraza-1,5-pentane diisocyanate, are prepared by reacting the corresponding diacyl halides, such as 4-nitraza-1,7-heptanediyl chloride, with an azide of an alkali or alkaline earth metal, such as sodium azide, and subsequently heating under anhydrous conditions to effect rearrangement to the desired diisocyanate, as more fully disclosed in assignee's copending U.S. patent application Serial No. 520,914, filed July 8, 1955.

40 It will be appreciated that a wide variety of bis-inorganic acid salts of nitraza diamines can be prepared in accordance with the method of my invention. For example, 3,6,9-trinitraza-1,11-undecane diisocyanate; 2,4-dinitraza-1,5-pentane diisocyanate; 2-nitrazapropane diisocyanate; and 3,5-dinitraza-1,7-heptane diisocyanate react with dilute nitric acid to produce the bis-nitric acid salts of the corresponding amines, namely, 3,6,9-trinitraza-1,11-undecane diamine; 2,4-dinitraza-1,5-pentane diamine; 2-nitrazapropane diamine; and 3,5-dinitraza-1,7-heptane diamine, respectively. Similarly, 3-nitraza-1,5-pentane diisocyanate; 2-nitraza-1,4-butane diisocyanate; and 3,10-dinitraza-1,12-dodecane diisocyanate react with dilute perchloric acid to yield the bis-perchloric acid salts of the corresponding amines, namely, 3-nitraza-1,5-pentane diamine; 2-nitraza-1,4-butane diamine; and 3,10-dinitraza-1,12-dodecane diamine, respectively.

45 It is apparent that any member of my new series of salts can be readily obtained by reacting the appropriate starting materials as taught herein.

This application is a continuation-in-part of my copend-

ing U.S. patent application Serial No. 451,709, filed August 23, 1954, now abandoned.

I claim:

1. As new compositions of matter, the bis-inorganic acid salts of nitraza diamines having the general formula: 5



wherein X is a radical selected from the group consisting of nitrate and perchlorate radicals; A and A' are lower alkylene radicals; and n is a whole number from 1 to 6, inclusive.

2. As new compositions of matter, the bis-nitric acid salts of nitraza diamines having the general formula: 10



wherein A and A' are lower alkylene radicals and n is a whole number from 1 to 6, inclusive.

3. As new compositions of matter, the bis-perchloric acid salts of nitraza diamines having the general formula: 15



wherein A and A' are lower alkylene radicals and n is a whole number from 1 to 6, inclusive.

4. As a new composition of matter, the bis-nitric acid salt of 3-nitraza-1,5-pentane diamine having the structural formula: 20



5. As a new composition of matter, the bis-nitric acid salt of 3,6-dinitraza-1,8-octane diamine having the structural formula: 25



6. As a new composition of matter, the bis-perchloric acid salt of 3-nitraza-1,5-pentane diamine. 30

7. As a new composition of matter, the bis-perchloric acid salt of 2-nitraza-1,4-butane diamine.

8. As a new composition of matter, the bis-perchloric acid salt of 3,10-dinitraza-1,12-dodecane diamine.

9. As a new composition of matter, the bis-nitric acid salt of 3,6,9-trinitraza-1,11-undecane diamine having the structural formula: 35



10. As a new composition of matter, the bis-nitric acid salt of 2,4-dinitraza-1,5-pentane diamine having the structural formula: 40



11. The method of preparing bis-inorganic acid salts of nitraza diamines having the general formula: 45



which comprises reacting a nitraza diisocyanate having the general formula:



with a dilute inorganic acid having the general formula HX; wherein X is a radical selected from the group consisting of nitrate and perchlorate radicals, A and A' are lower alkylene radicals, and n is a whole number from 1 to 6, inclusive.

12. The method of preparing bis-nitric acid salts of nitraza diamines having the general formula:



which comprises reacting a nitraza diisocyanate having the general formula:



with dilute nitric acid; wherein A and A' are lower alkylene radicals and n is a whole number from 1 to 6, inclusive.

13. The method of preparing bis-perchloric acid salts of nitraza diamines having the general formula:



which comprises reacting a nitraza diisocyanate having the general formula:



with dilute perchloric acid; wherein A and A' are lower alkylene radicals and n is a whole number from 1 to 6, inclusive.

14. The method of preparing the bis-nitric acid salt of 3-nitraza-1,5-pentane diamine which comprises reacting 3-nitraza-1,5-pentane diisocyanate with dilute nitric acid. 30

15. The method of preparing the bis-nitric acid salt of 3,6-dinitraza-1,8-octane diamine which comprises reacting 3,6-dinitraza-1,8-octane diisocyanate with dilute nitric acid. 35

16. The method of preparing the bis-perchloric acid salt of 3-nitraza-1,5-pentane diamine which comprises reacting 3-nitraza-1,5-pentane diisocyanate with dilute perchloric acid. 40

17. The method of claim 11 in which the dilute inorganic acid has a concentration of from about 30% to about 85%.

18. The method of claim 12 in which the dilute nitric acid has a concentration of about 35%.

19. The method of preparing bis-nitric acid salts of nitraza diamines having the general formula:



which comprises reacting a nitraza diisocyanate having the general formula:



with 35% nitric acid, in the presence of excess dilute nitric acid and at an elevated temperature; wherein A and A' are lower alkylene radicals and n is a whole number from 1 to 6, inclusive.

20. The method of preparing bis-nitric acid salts of nitraza diamines having the general formula:



which comprises reacting a nitraza diisocyanate having the general formula:



with 35% nitric acid, in the presence of dilute nitric acid and on a steam bath; wherein A and A' are lower alkylene radicals and n is a whole number from 1 to 6, inclusive.